

J. T. MARSHALL.  
MANUFACTURE OF LAMP FILAMENTS.  
APPLICATION FILED MAY 22, 1908.

996,420.

Patented June 27, 1911.



Witnesses:

Irving E. Stern

J. Eli Glen.

Inventor  
John T. Marshall.  
by Albert, Davis  
His Attorney.

# UNITED STATES PATENT OFFICE.

JOHN T. MARSHALL, OF METUCHEN, NEW JERSEY, ASSIGNOR TO GENERAL ELECTRIC COMPANY, A CORPORATION OF NEW YORK.

## MANUFACTURE OF LAMP-FILAMENTS.

996,420.

Specification of Letters Patent. Patented June 27, 1911.

Application filed May 22, 1908. Serial No. 434,215.

*To all whom it may concern:*

Be it known that I, JOHN T. MARSHALL, a citizen of the United States, residing at Metuchen, in the county of Middlesex, State 5 of New Jersey, have invented certain new and useful Improvements in the Manufacture of Lamp-Filaments, of which the following is a specification.

My present invention consists in an improvement in the manufacture of lamp filaments of that type commonly known to the trade as "metallized" filaments.

More specifically, my invention consists in so modifying the method of manufacture 15 that the resulting filaments are more dense, uniform, and homogeneous in structure and are more durable and efficient in operation.

The drawing illustrates diagrammatically apparatus that may conveniently be made 20 use of in the practice of my invention commercially.

My improved process contemplates the introduction of an additional step into the process of manufacturing the so-called metallized filaments, as previously practiced,—described in United States Patent No. 916,905, granted March 30, 1909 to Willis R. Whitney. It will be recalled by those skilled in the art that in the process referred to a "base 25 filament" of carbon (usually obtained by carbonization of a squirted filament of cellulose out of contact with the air) is fired to a very high temperature to remove impurities, given a carbonaceous coating by the 30 ordinary flashing or treating process of heating with current in benzin vapor, and fired to about the same temperature as before or to a higher temperature. This second heat treatment produces profound changes in the skin 35 or coating and yields the well-known high efficiency filament commonly designated as a "metallized" filament. This filament is composite, that is to say, it is a filament consisting really of two conductors in parallel, 40 a carbon base, and a shell or skin. The temperature resistance curve of the shell or skin is a curve characteristic of a metal conductor and very different from the curve of ordinary carbon. Without speculating 45 as to the nature of the changes which have gone on during this second firing, it is sufficient for the present purpose to note that great changes have taken place and the characteristics of the shell have been greatly

modified. Now it happens that this second 55 firing treatment, whereby the coating of graphite is metamorphosed into a different material, imposes severe strains on the composite filament and tends to break up the union between core and shell and to destroy 60 the homogeneous character of the conductor. It seems very possible that when the changes take place in the shell violent expansion and contraction may occur and even complete 65 molecular rearrangements, whereby the shell tends to separate from the core. At all events, I have found that in some cases it is possible to strip off sections of the shell or coating as little tubes. Furthermore, I have noticed that some filaments as they 70 come from this second firing, have the outer shell projecting slightly beyond the inner core at the end of the filament, much as if the shell had expanded more than the core and slipped out over the end. It is, of 75 course, possible that this peculiar effect is produced by shrinkage of the core, but at all events it represents a relative movement between the two portions of the filament and indicates the probability that they have been 80 torn apart by the violence of the high heat treatment.

Having described the characteristic features of the process by which metallized carbon filaments have heretofore been commercially manufactured, I will now proceed to indicate how this process can be improved, pointing out some of the advantages accruing from the improvement.

Briefly stated, the improvement consists 90 in so locking the shell to the inner core that relative movement between the two is impossible, and stripping or flaking of the shell does not occur. This result is effected by introducing into the process as above set 95 forth, an additional step having for its object the roughening of the core or base prior to its treatment in the benzin vapor, or in other words, prior to the deposition on it of the material which subsequently becomes 100 the metallized shell of the filament.

The roughening treatment above mentioned is effected by heating the core in the air for a brief time interval. This produces oxidation at the surface with resultant pitting and roughening. In practice I find it convenient to effect this oxidation or flashing in air by first mounting the filament f 105

on a treating cork C in the usual manner and then touching the terminals *t*, *t* against two contacts T, T across which a suitable potential is applied by some sort of an automatic timing device, such for instance as a spur *s* carried on a revolving shaft S, and at each revolution wiping across a spring K acting as a contact. The time of contact of the spur and spring should be a fraction 5 of a second and may be made adjustable by making the spring either nearer to or farther from the spur. In general, the time of treatments should be made long enough to increase the resistance of the filament about 10 25%. I have found that the voltage should be about three times the voltage which would be necessary to bring the filament to 3.1 watts per candle in a vacuum. This step 15 of flashing in air is the only change contemplated by me in the process of manufacturing metallized filaments. The treatment requires only a moment and yet the benefits are far reaching. For when the coating is put on the core by heating with current in 20 benzine vapor, the deposited material fills up the pits of the roughened core and takes such a grip on the core that it never works loose even under the action of those most powerful stresses set up by the very high 25 temperature of the second firing.

From a commercial standpoint the value 30 of my improvement resides principally in an increased life for the lamps, both as regards early breakage and average life. 35 In some instances the improvement has amounted to as much as 50% of the life of metallized filaments as heretofore made.

What I claim as new and desire to secure by Letters Patent of the United States, is—

1. As a step in the production of metallized carbon filaments, roughening the base before flashing in the volatile hydrocarbon. 40
2. As a step in the production of metallized carbon filaments, oxidizing the surface of the base subsequent to the first firing. 45
3. As a step in the production of metallized carbon filaments, oxidizing the fired base prior to flashing, by heating with an electric current in air. 50
4. As a step in the production of metallized carbon filaments, heating the base in air to roughen the surface and prevent subsequent slipping of the superimposed shell. 55
5. As a step in the production of metallized carbon filaments, subjecting the base to the action of a suitable reagent to roughen its surface prior to coating the same. 60
6. As a step in the production of metallized carbon filaments, subjecting the base to the action of an oxidizing agent prior to coating the same. 65
7. As a step in the production of a metallized carbon filament, roughening the base prior to coating and metallization.
8. As a step in the production of a metallized carbon filament, roughening a fired base prior to coating and metallization.

In witness whereof, I have hereunto set my hand this 19th day of May, 1908.

JOHN T. MARSHALL.

Witnesses:

S. N. WHITEHEAD,  
J. HARRY ELKINS.